

# UNITED STATES PATENT OFFICE.

WILLIAM G. HOUSKEEPER, OF NEW YORK, N. Y., ASSIGNOR TO WESTERN ELECTRIC COMPANY, INCORPORATED, OF NEW YORK, N. Y., A CORPORATION OF NEW YORK.

## LEADING-IN WIRE.

1,357,498.

Specification of Letters Patent.

Patented Nov. 2, 1920.

No Drawing.

Application filed November 25, 1919. Serial No. 340,669.

To all whom it may concern:

Be it known that I, WILLIAM G. HOUSKEEPER, a citizen of the United States, residing at New York, in the county of New York, State of New York, have invented certain new and useful Improvements in Leading-in Wires, of which the following is a full, clear, concise, and exact description.

This invention relates to leading-in wires 10 for incandescent lamps, vacuum tubes, mercury arc rectifiers and the like, and more particularly it relates to a method of coating base metal leading-in wires with a fluxing material.

15 The object of this invention is to produce a leading-in wire having superimposed upon it a flux-containing composition of sufficient elasticity and toughness to withstand any bending or twisting incident to the reeling 20 of the wire.

In making use of iron, iron nickel alloy and copper wires for conducting current through the glass walls of evacuated glass articles, it has been found desirable to employ 25 a fluxing agent in order to secure a satisfactory tight seal. While the fluxing medium may be applied just prior to the insertion of the wire in the glass, it is highly desirable that a continuous film of the flux be 30 so attached to the wire as to allow the latter to be reeled, subsequent to the treatment, without danger of disrupting the superimposed coating.

A suitable material which can be removed 35 easily by the aid of heat is to be preferred in binding the flux to the wire. Organic compounds which contain no metallic radical are admirably adapted for this purpose. Some of the organic substances which are 40 suitable for use contain water either as water of combination or constitution, which, however, will not be detrimental to the subsequent use and treatment to which the coating is subjected.

45 Such a film or coating is produced, according to this invention, by adding to the flux a suitable colloid-forming material which is capable of forming a hard, continuous layer on a metallic surface. As a flux medium a 50 borate, for example borax  $Na_2B_4O_7 \cdot 10H_2O$  is preferably used. To this in concentrated solution is added a predetermined amount of a suitable colloid-forming material, as, for example, gelatin. The wire to be cov- 55 with this composition is first freed from any

surface grease or dirt and then passed slowly through the bath. As it comes out of the latter the coating is dried in a current of warm, dry air. This process produces a tough, elastic coating, and consequently the 60 wire may be reeled and kept until needed; and may be shipped and handled without danger of injury to the coating. During the sealing-in process when the heat applied reaches a certain temperature, the organic 65 material is decomposed, the volatile matter being volatilized, and the carbon uniting with the oxygen of the warm air to form the gaseous oxids of carbon.

While gelatin has been mentioned as the 70 colloid-forming material which is preferred for use in the process, it is to be understood that any colloid-forming material having the properties of gelatin, when used in the manner described above, and any borate 75 having the fluxing properties of borax may be employed.

It may sometimes be desirable to add glycerin to the bath in order to prevent the borax from crystallizing out. This addition would be required where the bath becomes over concentrated due to the loss of water. The presence of glycerin in the bath will, moreover, have a beneficial effect if the wire is to be stored a considerable length of 85 time after treatment.

What is claimed is:

1. The method of producing a superimposed flux coating on a leading-in wire which consists in drawing the wire through 90 a bath containing a borate and a colloid-forming material and then subjecting it to a current of warm, dry air.

2. A leading-in wire covered with a composition containing a borate, and a carbonaceous binder, with or without  $H_2O$ . 95

3. A leading-in wire covered with a composition containing a borate and a colloid-forming material.

4. A leading-in wire covered with a composition containing glycerin, a borate and a colloid-forming material. 100

5. A leading-in wire covered with a composition containing a borate and gelatin.

6. A leading-in wire covered with a composition containing borax and gelatin.

In witness whereof, I hereunto subscribe my name this 20th day of November, A. D. 1919.

WILLIAM G. HOUSKEEPER.